

## UNITED STATES PATENT OFFICE

WALLACE HENRY PAULL AND REGINALD TRUESDALE, OF FORT DUNLOP, BIRMINGHAM, ENGLAND, ASSIGNEES TO DUNLOP TIRE AND RUBBER CORPORATION OF AMERICA, OF BUFFALO, NEW YORK, A CORPORATION OF NEW YORK

## MANUFACTURE OF YARN

No Drawing. Application filed October 27, 1926, Serial No. 144,642, and in Great Britain November 28, 1925.

This invention relates to improvements in the manufacture of yarns, and has particular reference to yarns of composite construction.

Such yarns necessarily possess the characteristics of their component fibers and it is the object of the present invention to combine into a yarn fibers which will characterize the same at once with great strength and pleasing appearance and finish.

10 According to this invention we produce a yarn by mixing ramie or rhea fiber with artificial silk fiber prepared by any of the known processes, for example, the viscose, cellulose acetate, cupro-ammonium or nitro-cellulose processes.

The yarn may be produced by mixing in suitable proportion and spinning together the natural ramie or rhea fiber and the artificial silk fiber.

20 The proportions in which the fibers are mixed depends on the purpose for which they are required. A yarn for use in cord fabric for tires may consist of approximately 75% ramie or rhea fiber and 25% artificial silk fiber.

The yarn may also be produced by spinning the artificial silk fibers and the ramie fibers together separately into thread and then doubling the threads together in suitable proportions, which may, for example, be the proportions indicated above.

30 It will be apparent that the practice of the invention does not necessarily demand the utilization of any special or particular kind of apparatus, it being understood that standard textile machinery may be used to carry out all the required steps of the process of the said invention.

The ramie or rhea fiber is of great strength 40 but lacks flexibility whereas the artificial silk fiber is extremely flexible but relatively weak. A mixture of the two in suitable proportions is extremely suitable for our purpose.

45 By thus combining the artificial silk or rayon and ramie fibers and spinning them together into thread and doubling, a cord will be obtained that has a resistance to fatigue much greater than that of other fibers heretofore available and which, therefore, forms with the rubber in which it is embedded a

more durable and better wearing tire structure.

Having now particularly described and ascertained the nature of our said invention and in what manner the same is to be performed we declare that what we claim is:

55 1. A cord tire for vehicle wheels having cords composed of fibrous ramie and artificial silk.

2. A cord tire for vehicle wheels having cords composed of about 75% of ramie fibres and 25% artificial silk fibres.

3. A cord tire for vehicle wheels having cords composed of spun and twisted fibers of ramie and artificial silk embedded therein.

65 In witness whereof, we have hereunto signed our names.

WALLACE HENRY PAULL.  
REGINALD TRUESDALE.

70

75

80

85

90

95

100